

# UNITED STATES PATENT OFFICE.

SYDNEY SMITH, OF DETROIT, MICHIGAN, ASSIGNOR TO THE STUDEBAKER CORPORATION, A CORPORATION OF NEW JERSEY.

## METHOD OF TREATING WOOD.

Patented June 7, 1921.

1,380,429.

Specification of Letters Patent.

No Drawing.

Application filed August 2, 1919. Serial No. 315,035.

To all whom it may concern:

Be it known that I, SYDNEY SMITH, a citizen of the United States of America, and resident of Detroit, in the county of Wayne 5 and State of Michigan, have invented certain new and useful Improvements in Methods of Treating Wood, of which the following is a specification.

This invention relates to a method or 10 process for the treatment of wood whereby it is conditioned to withstand high temperatures in excess of its normal critical point and whereby its strength is increased.

When different kinds of woods are subjected to a rise in temperature it is found that each particular kind will withstand a certain degree of temperature rise without showing any deleterious effect, whereas, a continued rise in temperature above this 20 point will result in the destroying of the wood fibers, charring of the wood and depreciation in the strength thereof. The temperature at which the wood succumbs to the heat varies with different woods, and the 25 point at which any particular kind of wood begins to be seriously affected by heat is known as the critical point. In practice, it is found that for the well known woods this temperature will vary from between 125 30 degrees F. to 160 degrees F.

It is desirable at times in the various arts to so condition wood that it will be able to withstand high temperatures in excess of the normal critical points of the particular 35 kind of wood employed. For the purposes of this disclosure, it is not necessary here to specify the particular arts or the uses to which the wood is employed, but it is sufficient to note that frequently it is desirable 40 to provide means whereby the critical point of a particular kind of wood may be so raised that it may be subjected to otherwise excessive heat without deleterious effects upon the wood. It is also an advantage to increase 45 the strength of the wood for certain uses.

With the purpose of accomplishing these results, I have treated several species of wood by the process hereafter described, and I have discovered that said critical point is 50 raised by such treatment and the strength of the wood is increased.

My method or process consists in treating wood with a solution by immersion or by coating, and then subjecting the wood thus 55 treated to heat, the heat being applied with

a slow but regular rise in temperature from zero to approximately two hundred degrees F., extending over a period of approximately four hours. The solution that I have employed for treating wood is what is known 60 in the market as Standard grip enamel. I have found that satisfactory results are accomplished with this substance, but there are other substances of a kindred nature, that is enameling fluids, having the same general 65 chemical constituents, which no doubt would serve the same purpose.

My experiments have demonstrated that wood, the normal critical point of which is around 150 degrees F., can, after being treated as described, be safely subjected to a temperature upward of 300 degrees F. without any detrimental effects. In fact, the treatment serves to not only protect the wood 70 against temperature rise, but also serves to 75 impart greater strength to the wood than was present therein prior to the treatment.

For the purpose of illustration, the result of one experiment will suffice. A piece of maple without any treatment whatsoever 80 was subjected to a heat test and its critical point was found to be around 160 degrees. The second piece of maple, cut adjacent the first piece, and of the same size, was treated 85 in accordance with the method of this invention, the slow baking operation extending over a period of four hours and the maximum temperature reached being 200 degrees F. This latter piece of maple, treated as described, was later subjected to 90 upward of 275 degrees F. without showing any deleterious effect. In this experiment the treated wood withstood an increased rise of 115 degrees above its normal critical 95 point as a result of said treatment. A strength test was also made on both of these pieces of maple, and it was found that the untreated piece broke at 940 pounds. When the treated wood was subjected to a breaking strain it was found to break at 1530 100 pounds. It thus appears that in the experiment referred to, the wood which had undergone the treatment of this process withstood a test of nearly 600 pounds greater than the untreated stock, or, in round numbers, its strength had been enhanced through the treatment approximately two-thirds.

Thus the method or process operates not only to raise the critical point of wood but to greatly increase the strength thereof. 110

In the foregoing description, I have specifically set forth and described the preferred manner of practising the invention, but it will be understood that I do not limit the method to the specific materials or temperatures specified. The substitution of equivalents and the varying of the temperatures in accordance with the particular woods under consideration are within the scope of this invention.

What I claim is:

1. In the art of treating wood, the process of increasing its strength and raising its critical point, which consists in applying to the wood a chemical agent and thereafter subjecting it to a gradual rise in temperature extending over a prolonged period.
2. In the art of treating wood, the process of increasing its strength and raising its critical point, which consists in applying to the wood a chemical agent and then subjecting it to a gradual rise in temperature extending over a prolonged period, during which a temperature at least equal to the critical point of the wood treated is attained.
3. In the art of treating wood, the process of increasing its strength and raising its

critical point, which consists in applying a chemical agent to the wood and thereafter subjecting it to a gradual rise in temperature over a period of upward of three hours, during which a temperature upward of the temperature of the critical point of the wood treated is attained.

4. In the art of treating wood, the process of increasing its strength and raising its critical point, which consists in applying a chemical agent to the wood, and thereafter subjecting it to a gradual rise in temperature for a period of approximately four hours during which a temperature of approximately 200° F. is attained.

5. In the art of treating wood, the process of increasing its strength and raising its critical point, which consists in applying thereto an enameling fluid and thereafter subjecting it to a gradual rise in temperature.

Signed by me at Detroit, Michigan, U. S. A. this 29th day of July, 1919.

SYDNEY SMITH.

Witnesses:

VINCENT LINK,  
A. E. LEACH.